

June 1, 1971

A. GOTTLIEB ET AL

3,581,366

THERMOSTATIC BIMETAL

Filed Dec. 9, 1968



FIG. 1



$\frac{1}{10} \cdot 01 = 0.01 \text{ IN. DEF. IN } 400^{\circ} \text{ F. } - 50^{\circ} \text{ F. } = 0.07$

FIG. 2

INVENTORS  
ARNOLD J. GOTTLIEB  
GEORGE A. MAJESKO  
BY  
Theodore J. Jugh  
ATTORNEY

## 1

3,581,366

## THERMOSTATIC BIMETAL

Arnold Gottlieb, Colonia, and George A. Majesko, Glen Ridge, N.J., assignors to Wilbur B. Driver Company  
Filed Dec. 9, 1968, Ser. No. 782,070  
Int. Cl. B32b 15/00

U.S. CL. 29—195.5

2 Claims

## ABSTRACT OF THE DISCLOSURE

A thermostatic bimetal having enhanced temperature dependent characteristics such as the amount and linearity of deflection and developed force as well as an extended temperature range of maximum sensitivity. The bimetal employs a low expanding component containing, as major constituents, 30.75%—31.75% by weight of nickel, 6.5%—8.5% of cobalt, balance iron. This component can also contain, as minor constituents, manganese, carbon and silicon.

## SUMMARY OF THE INVENTION

All thermostatic bimetals possess certain important characteristics which are functions of temperature; i.e., the amount and linearity of deflection, the amount and linearity of developed force, and the range of maximum sensitivity. (This range is the temperature range of maximum rate of change of deflection and force.) All of these characteristics are related to  $\Delta\alpha$ , which is the difference between the coefficients of thermal expansion of the high and the low expanding components of the bimetal. The standard low expanding component is Invar, which uses two major constituents, nickel (.36% by weight) and iron.

In contradistinction, we employ as a low expanding component an iron-nickel-cobalt alloy having the following composition, by weight:

|        | Percent     |
|--------|-------------|
| Nickel | 30.75—31.75 |
| Cobalt | 6.5—8.5     |
| Iron   | Balance     |

In addition, this alloy can contain 0.05%—0.50% of manganese and .015%—0.12% of carbon. Further, this alloy can also contain .015%—0.15% of silicon. The  $\Delta\alpha$  attained from thermostatic bimetals using this alloy is larger than any other bimetal using Invar and moreover, the linearity of  $\Delta\alpha$  is maintained within desired limits over a greater temperature range. As a result, our bimetal, for a given temperature range, is characterized by enhanced magnitude and linearity of both force and deflection as well as an extended range of maximum sensitivity.

## BRIEF DESCRIPTION OF THE DRAWINGS

In the drawings:

FIG. 1 is a perspective view of a bimetal in accordance with our invention; and

FIG. 2 is a graph comparing the change of  $\Delta\alpha$  with temperature of certain of our bimetals as compared to a bimetal using Invar.

## DETAILED DESCRIPTION OF PREFERRED EMBODIMENT

FIG. 1 shows a typical bimetal in accordance with our invention having two bonded layers 10 and 12. Layer 10 is a conventional high expanding component such as chromium-nickel-iron. Layer 12 is a low expanding component in accordance with our invention.

The overall composition ranges of the major constitu-

## 2

ents of this low expanding component as expressed in percent by weight are:

|        | Percent     |
|--------|-------------|
| Nickel | 30.75—31.75 |
| Cobalt | 6.50—8.50   |
| and    |             |
| Iron   | Balance     |

The ranges of the minor constituents of this component are:

|           | Percent    |
|-----------|------------|
| Manganese | 0.05—0.50  |
| Carbon    | 0.015—0.12 |
| Silicon   | 0.015—0.15 |

No special processing is required in using this alloy together with other bimetal alloys as compared to using standard Invar. Conventional hot and cold bonding techniques may be used together with standard annealing and cold rolling procedures.

The important thermostatic bimetal characteristics of curvature (reciprocal of radius of curvature), deflection and force are functions of  $\Delta\alpha$  (the difference in expansion coefficients of the high and low expanding elements), as well as the thicknesses of these components and the ratio of the elastic moduli of the low expanding and high expanding components. Since the modulus of our low expanding alloy is approximately the same as that of standard Invar and the thickness is a design consideration only,  $\Delta\alpha$  is the most important parameter.

A known bimetal using Invar as the low expanding component and a known nickel-chromium-iron high expanding component (typical composition 22% by weight of chromium, 3% nickel, balance iron) was prepared, and its  $\Delta\alpha$  was measured and plotted as a function of temperature as shown at curve 20 in FIG. 2.

Two bimetals using the same high expanding component and two different compositions of our low expanding alloy were prepared and the two different  $\Delta\alpha$ 's were measured and plotted as a function of temperature as shown at curves 22 and 24 respectively in FIG. 2.

The low expanding alloy used in obtaining curve 22 had the following composition:

|           |       |
|-----------|-------|
| Nickel    | 31.29 |
| Cobalt    | 7.05  |
| Manganese | 0.10  |
| Carbon    | 0.037 |
| Silicon   | 0.10  |

The low expanding alloy used in obtaining curve 24 had the following composition:

|           |       |
|-----------|-------|
| Nickel    | 31.54 |
| Cobalt    | 8.16  |
| Manganese | 0.07  |
| Carbon    | 0.016 |
| Silicon   | 0.10  |

It can be seen that the  $\Delta\alpha$  for each of curves 22 and 24 is not only larger than that for curve 20, but is also more nearly constant with increasing temperature. Note that curves 22 and 24 have a spread in  $\Delta\alpha$  of  $.50 \times 10^{-6}/^{\circ}\text{F.}$  and  $.20 \times 10^{-6}/^{\circ}\text{F.}$  respectively as compared to a spread of  $.90 \times 10^{-6}/^{\circ}\text{F.}$  for curve 20 over the temperature range of  $100^{\circ}\text{—}500^{\circ}\text{F.}$

The flexibility coefficient is a fundamental parameter for evaluating bimetal characteristics. It is the temperature coefficient of curvature defined as:

$$F = \frac{\left(\frac{1}{R_2} - \frac{1}{R_1}\right)t}{T_2 - T_1}$$

where:

$F$ =Flexivity

$R_1$ =Radius of curvature at temperature  $T_1$

$R_2$ =Radius of curvature at temperature  $T_2$

$t$ =Thickness of bimetal

The following table compares the flexivity coefficients that can be obtained with the compositions such as used for curves 22 and 24 as compared with the known composition of curve 20. The temperature range for flexivity measurement is 100° F.-300° F. and the two components have equal thicknesses.

### FLEXIVITIES

[Parts per million per degree F.]

Over the temperature range of 100° F.-300° F.

|          |      |
|----------|------|
| Curve 20 | 14.6 |
| Curve 22 | 15.7 |
| Curve 24 | 15.3 |

Greater increases in flexivity can be obtained when high expanding elements having lower expansion coefficients than that used herein are coupled without low expanding alloy.

As a result, our bimetals, as compared to known bimetals, are characterized by:

- (1) Greater deflection for a given temperature change because of a larger value of  $\Delta\alpha$ ;
- (2) Greater force for a given temperature change because of a larger value of  $\Delta\alpha$ ; and
- (3) Enhanced linearity of deflection and force with temperature, and greater temperature range of maximum sensitivity due to a more uniform value of  $\Delta\alpha$  over a larger temperature range.

Within the normal operating temperature range of bimetals, the composition ranges given herein result in the

optimization of  $\Delta\alpha$  and the temperature range of maximum sensitivity.

While we have described our invention with particular reference to preferred embodiments, our protection is to be limited only by the scope of the claims which follow.

5 What is claimed is:

1. A thermostatic bimetal comprising: first and second metallic layers bonded together to define a strip, the first layer being a high expanding alloy, the second layer being a low expanding alloy, said strip being characterized by a parameter,  $\Delta\alpha$ , which is the difference between the thermal coefficients of expansion of the two layers, said parameter having a substantially constant value over a temperature range of 100° F. to 300° F. and being in excess of  $1.01 \times 10^{-7}$  per ° F. throughout this range; said first layer consisting essentially of nickel, chromium and iron; said second layer consisting essentially of the following as expressed in percent by weight:

|           | Percent     |
|-----------|-------------|
| Nickel    | 30.75-31.75 |
| Cobalt    | 6.5-8.5     |
| Manganese | 0.05-0.5    |
| Carbon    | 0.015-0.12  |
| Silicon   | 0.015-0.15  |
| and       |             |
| Iron      | Balance     |

2. A bimetal as set forth in claim 1 wherein the first layer consists essentially of 22% chromium, 3% nickel, balance iron.

### References Cited

#### UNITED STATES PATENTS

|           |         |          |          |
|-----------|---------|----------|----------|
| 1,604,064 | 10/1926 | Miller   | 29—195.5 |
| 1,689,814 | 10/1928 | Brace    | 29—195.5 |
| 2,941,882 | 6/1960  | Franklin | 75—123   |

HYLAND BIZOT, Primary Examiner

UNITED STATES PATENT OFFICE  
CERTIFICATE OF CORRECTION

Patent No. 3,581,366 Dated June 1, 1971

Inventor(s) Arnold Gottlieb and George A. Majesko

It is certified that error appears in the above-identified patent and that said Letters Patent are hereby corrected as shown below:

Column 1, line 34 of the specification (.36% by weight) should read--(36% by weight)--.

Signed and sealed this 21st day of December 1971.

(SEAL)

Attest:

EDWARD M.FLETCHER, JR, JR.  
Attesting Officer

ROBERT GOTTSCHALK  
Acting Commissioner of Patents